

Patented Nov. 20, 1928.

1,692,690

# UNITED STATES PATENT OFFICE.

SIDNEY OSSER, OF WICHITA, KANSAS.

## RAPID MAGNETIZING AND DEMAGNETIZING METAL ALLOYS.

No Drawing.

Application filed June 26, 1926. Serial No. 118,640.

This invention relates to metal alloys and particularly to a metal alloy especially designed and adapted for use in the construction of electromagnets, transformers and other electrical instruments or devices.

The main object of the invention is to provide a metal having certain peculiarities of action rendering it of great value and importance in the construction and operation of electrical instruments of the class described, whereby the efficiency of such devices or instruments may be increased, to wit, a metal having extremely rapid magnetizing and demagnetizing qualities and which is capable of high saturation with low reluctance and, when demagnetized, of being devoid or substantially devoid of residual magnetism.

A further object of the invention is to provide a rapidly magnetizing and demagnetizing metal alloy which possesses proper relative degrees of hardness and ductility for the purpose, which may be manufactured and sold at a comparatively low cost, and which when machined or worked in any of the usual ways will take a very smooth finish.

In carrying my invention into practice I provide a metal alloy which may vary to certain degrees in the proportions of some or all of the ingredients employed, but the following composition gives very satisfactory results:

|                              |        |
|------------------------------|--------|
| Carbon                       | 12     |
| Manganese                    | .51    |
| Phosphorus                   | .103   |
| Sulphur                      | .090   |
| Silicon                      | .03    |
| Balance iron (substantially) | 99.147 |

In this composition the phosphorus gives a desired degree of hardness, and the manganese, in the proportion employed, gives the requisite degree of toughness without impairment of relative magnetizing and demagnetizing efficiencies. It is desirable, however, to keep the proportion of manganese content as low as possible, consistent with the production of a good working metal, in order to secure the advantage of its magnetic qualities to a certain degree, while preventing undesirable reluctance or other retardance actions interfering with rapid magnetization of the metal to a high saturation point and its rapid demagnetization at which practically no residual magnetism exists.

The sulphur in this composition exists as an

unavoidable impurity, and the same is largely true of the carbon, although in the use of certain grades of iron carbon up to the amount named may be used for its hardening effect. 60 The sulphur and carbon content, however, should be kept as low as possible, as these elements are of no particular importance so far as the electrical qualities of the metal are concerned. The silicon gives ductility 65 and renders the metal readily annealable. The combination of iron, manganese, phosphorus and silicon, combined in the proportions or substantially in the proportions named, gives to this metal the novel and peculiar electrical qualities especially adapting it for use in electrical instruments or devices of the character set forth. While the proportions set forth are preferred they may be varied to certain degrees, particularly with 70 regard to the silicon and phosphorus, without unduly changing the electrical efficiency of the metal. Thus, for example, the proportions of the phosphorus may vary from .103% to .15% or more, and the silicon from .03% 80 to .10% or more, without undesirably changing the physical or electrical qualities of the metal.

The metal alloy resulting from the combination of the constituents noted is a magnetic metal having the peculiar property of becoming magnetized with great rapidity under the influence of an electric current and of becoming rapidly demagnetized when the flow of current is arrested, these actions occurring with much greater rapidity than is possible with any other metal with which I am familiar. Practical demonstrations show that it has a rapid and high saturation factor combined with very low reluctance and practically no residual factor, making it very valuable for use in electromagnets, transformers and other electrical instruments and devices for rapid energizing and deenergizing actions and the avoidance of retardance 90 actions of various kinds. It may be cast, rolled or otherwise formed into shape, readily annealed, easily machined or otherwise worked, will take a smooth finish, and may be produced at a comparatively low cost. 95

Having thus fully described my invention, I claim:

1. A rapidly magnetizable and demagnetizable metal alloy resulting from a combination of or including iron, manganese, 110 substantially .51%, phosphorus, from .10% to .15%, and silicon, from .3% to .5%, and

iron sufficient in quantity to make the other ingredients according to the percentages employed 100%.

2. A metal alloy of the character and for the purpose described formed from a combination of carbon .12%, manganese .51%, phosphorus .103%, sulphur .090%, silicon .03%, and iron 99.147%.

3. A metal alloy of the character and for

the purpose described formed from a combination of carbon, about .12%, manganese, about .51%, phosphorus, from .10% to .15%, sulphur, about .090%, silicon, from .3% to .5%, and iron sufficient in quantity to make with the other ingredients according to the 15 percentages employed 100%.

In testimony whereof I affix my signature.  
SIDNEY OSSER.